

# UNITED STATES PATENT OFFICE.

CHARLES C. HUFFMAN, OF CHICAGO, ILLINOIS, ASSIGNOR TO SUNBEAM CHEMICAL COMPANY, OF CHICAGO, ILLINOIS, A CORPORATION OF ILLINOIS.

## UNIVERSAL BLUE DYE AND METHOD OF PRODUCING THE SAME.

1,274,046.

Specification of Letters Patent. Patented July 30, 1918.

No Drawing.

Application filed September 24, 1917. Serial No. 192,871.

To all whom it may concern:

Be it known that I, CHARLES C. HUFFMAN, a citizen of the United States, and resident of Chicago, in the county of Cook and State 5 of Illinois, have discovered a certain new and useful Universal Blue Dye and Methods of Producing the Same, of which the following is a specification.

My discovery relates to dyes and particularly to a novel dye soap having peculiar and advantageous qualities.

I am aware that heretofore dyes have been incorporated in soaps with the object in view of providing a simple carrier for the dye and 15 fairly satisfactory results may be secured if neutral dyes are employed and if the water in which the substance is used is of exactly the right temperature.

My improved dye soap should not be confused with those in which the soap acts merely as a carrier or vehicle for the dye, as the following description will show that the final product is the result of peculiar reactions which take place between the dye and 25 the elements of the soap and which product could not be secured by the use of the materials heretofore employed or as heretofore combined. By reason of the novel process of compounding and the selection of substances which enter into the compound, a dye 30 is produced which is equal if not superior to those which require boiling and the addition of a mordant for setting the color.

One of the important distinctions of the 35 dyes produced by me is that they are alkali proof, irrespective of the characteristic of the dye, that is, basic, neutral or acid, before combining in the soap.

A still further distinction is that the dyes 40 are universal, that is, adaptable to either cotton, wool, silk or flax, or mixtures thereof.

One of the important advantages following the use of the method disclosed is that of allowing the glycerol, which is a by-product of the saponification process, to remain in the product. This is liberated when the soap is dissolved and coöperates with the dye in attacking the fabric. Furthermore it assists in fixing the colors following 45 the application of heat, as in the act of ironing, after the fabric has been dried.

The composition and the method of preparing it will now be described in detail.

In order to establish a basis for the 50 proportions of ingredients, it will be assumed

that it is desired to produce five gross of one ounce bars of the soap. To produce this quantity, three gallons and forty-two ounces of vegetable oil and one gallon and twenty-four ounces of sodium hydroxid ( $NaOH$ ) of a specific gravity of 1.40 at  $65^{\circ}$  F. are combined. The oil or oils used may be varied. Olive, soy bean, raisin, peanut, crude corn or any vegetable oil may be used separately or combined with cocoanut oil. The 60 proportions of the cocoanut oil and other oils will vary according to weather conditions. Under normal conditions one gallon, fourteen ounces of cocoanut oil will be employed to two gallons, twenty-eight ounces of the other oils. In warm, dry weather the proportion of cocoanut oil should be lessened and increased in cool, damp weather.

The oil and caustic soda are mixed until the saponification is nearly completed at 75 which time the dye solution is added. For the production of the various shades of blue a quantity of methylene blue or tetramethylionin chlorid ( $N(C_6H_5)_2S(N(CH_3)_2)_2Cl$ ) is dissolved in one gallon of boiling water 80 and is added to the mixture just described. The addition of this hot solution to the soap compound, together with the heat of the subsequent reaction, raises the temperature of the solution to approximately  $122^{\circ}$  F. at 85 which temperature the excess of sodium hydroxid reacts with the methylene blue forming a complex dye compound which differs from alkali blue in that it requires no developing. It also differs from methylene 90 blue as the latter is fast or permanent only on vegetable fibers whereas the compound produced is universal. The exact chemical formula of the product has not been determined and it can be defined only by reference to the materials entering into it and the method of combining them.

After allowing a few minutes for the reaction to take place and after the dye has become thoroughly mixed with the soap, the 100 soap is poured into molds where it is allowed to remain at a temperature of about  $80^{\circ}$  F. for forty-eight hours.

It will be noted that the glycerol is not removed from the product and therefore will be released as the soap is dissolved. It will be absorbed by the fabric along with the dye and will assist in fixing the dye when heat is applied to the fabric as in ironing. It has furthermore, an advantageous effect on the 105 110

fabric in softening the same and brightening the colors.

It will also be noted that no proportion of the methylene blue has been specified. The amount employed will vary with the shade desired as all the different shades from a baby blue to a dark blue may be secured by varying the quantity of methylene blue in the original compound. The amount necessary to produce the shade substantially midway between these two extremes is six ounces avoirdupois.

By comparison of the proportions of vegetable oil and sodium hydroxid it will be noticed that there is a substantial excess of the latter even when the water containing the dye is added. Of course, the amount of the saponifying agent may be varied somewhat but in any case an excess should be employed.

In use the soap and the garment or fabric to be dyed are introduced into hot water and the soap is applied directly to the fabric to thoroughly cleanse the same. Even though the soap is applied locally or only in spots the coloring will be even. Furthermore, the hands or container will not be colored. After the article is cleansed and dyed it is rinsed in cold water and dried in the usual manner. The dye will be found to be alkali proof.

One of the most important features of my novel discovery is that the shade of color which is secured in the use of the article is the same whether a large or small quantity is employed and whether it is used in hot or cold water. It is preferably used with hot water for the reason that the soap will not act to thoroughly cleanse the article unless the water is hot. The effect of deepening the shades by the use of hot water is not present and this is of great importance if it be desired to reproduce certain colors. The ordinary user has no means of determining whether the same temperature is employed in each instance. Neither would he be able to determine whether exactly the same quantity of the dyeing material was employed. By the use of my product the colors may be duplicated with ease and certainty.

Attention is called to the fact that the soap is manufactured by the cold process. By reason of this process of manufacture I am enabled to secure an absolutely uniform product with regard to the colors produced. The low temperatures employed are much more easily controlled and the necessary reaction between the soap and the dye is completed with a certainty which is not possible in a settled soap.

I claim:

1. The herein described universal blue dye which is formed by adding dissolved methylene blue to a saponified solution containing an excess of sodium hydroxid, substantially as described.

2. A blue dye soap composed of the reaction products of a vegetable oil, an excess of a saponifying agent, and a methylene blue, combined as set forth, substantially as described.

3. The method of producing a universal, alkali proof blue dye combined with soap which consists in combining a vegetable oil and a quantity of sodium hydroxid in excess of that required for saponification, then dissolving methylene blue in hot water and adding the dye solution to the saponified solution just before saponification is completed, then thoroughly mixing and then molding the soap, substantially as described.

4. The method of producing a universal blue combined with soap, which consists in preparing a solution of vegetable oil and an excess of sodium hydroxid, then dissolving methylene blue in boiling water and adding the same to the soap solution, the heat of the bodies plus the heat of the subsequent reaction being such as to bring the temperature of the compound to approximately 122° F., then pouring the material, substantially as described.

5. The method of producing an alkali proof, universal dye combined with soap, which consists in saponifying a vegetable oil with a substantial excess of the saponifying agent, then dissolving methylene blue in water and adding the same to the soap solution prior to the complete saponification and without removal of glycerol from the soap, the temperature of the compound after the addition of the dye being raised to substantially 122° F., then allowing the reaction to be completed and finally allowing solidification, substantially as described.

6. A dye soap formed by combining approximately four hundred and twenty-six parts of a vegetable oil and one hundred and fifty-two parts of sodium hydroxid of a specific gravity of 1.40 at 65° F., then adding to the compound just prior to complete saponification, one hundred and twenty-eight parts of hot water in which substantially six ounces of methylene blue has been dissolved, substantially as described.

Signed at Chicago, Ill., this 22nd day of September, 1917.

CHARLES C. HUFFMAN.

Witness:

T. D. BUTLER.